

## UNITED STATES PATENT OFFICE

1,969,018

## ALLOY

Robert H. Leach, Fairfield, Conn., assignor to  
Handy & Harman, New York, N. Y., a corpora-  
tion of New York

No Drawing. Application June 10, 1932,  
Serial No. 616,498

4 Claims. (Cl. 75—1)

This invention relates to silver alloys and is concerned more particularly with a novel silver alloy which may be used to especial advantage in the manufacture of table silver and hollow ware and for various other purposes, because it has the property of strongly resisting tarnish and discoloration.

As is well known, silver alloys of ordinary composition and containing copper as the base ingredient are susceptible to tarnish. Such discoloration of the metal is brought about by numerous agents, the most active being sulphur which is present in various foods such as eggs, and is also present to some extent in the atmosphere in the form of gaseous compounds. Sulphur in both forms causes tarnishing at a rate which depends on the length of contact or exposure of the metal, the concentration of the sulphur in the food or air, and the form in which the sulphur is present. In any event, the necessity of frequent cleaning and polishing of silver articles to keep them in bright condition has led to numerous attempts in the past to produce silver alloys which are of good appearance, have the desired working characteristics, and have a better resistance to tarnish than ordinary silver-copper alloys, but up to the present, the proposed alloys with which I am familiar, have not proven entirely satisfactory.

The problem of producing a silver alloy which is resistant to tarnish is a difficult one because investigation has shown that binary alloys offer little promise and the number of ternary and quaternary alloys is very large. When it is understood that small variations in the ingredients in these alloys have an important effect on the resistance to tarnish and the amounts of the alloying ingredients used are highly critical with respect to tarnish resistance, the magnitude and difficulty of the problem will be appreciated.

As a result of my investigations in this field, I have found that a silver alloy which has excellent resistance to tarnish produced by various agencies may be produced by using cadmium and tin as alloying metals, provided the cadmium and tin are confined within rather narrow limits, and the new alloys may be given a somewhat improved resistance to tarnish and, in some cases better physical properties, if a small amount of a fourth ingredient is added, which may be one or more of the metals, nickel, silicon, antimony and magnesium. In most instances, the fourth ingredient has a slight hardening effect and I shall, therefore, refer to it as a "hardener", although it is to be understood that not all of the metals mentioned

in this group have that effect. All the metals in the group, however, do increase the tarnish resistance to a greater or less degree. Of the several metals mentioned for use as hardeners, I prefer to use nickel, as it offers certain advantages over the others in the group. However, for the purpose for which these metals are used in the new alloy, all four metals are substantial equivalents.

Silver alloys which are now in widest use are those of sterling fineness containing not less than 925 parts of silver per thousand, and in producing the new alloy of sterling fineness, I use approximately 92.5% silver, cadmium ranging from about 3% to about 4%, tin ranging from about 3% to 4½%, and a small amount of nickel, silicon, antimony, and/or magnesium as a hardener, nickel and/or silicon being especially desirable as hardening ingredients. When any one of the hardening metals is used, the amount present is from about ½% to not to exceed about 1%, but when two or more are employed, the total amount of the hardening ingredients is not to exceed about 1.5%.

Instead of using cadmium as an element in the new alloy, I have found that approximately the same results may be obtained if zinc be substituted for part or all of the cadmium. I prefer to use cadmium, however, and believe that the resistance to tarnish of the new alloy in which cadmium is used instead of zinc is somewhat greater than that of an alloy in which zinc is present.

Typical examples of the new alloys of sterling fineness have the following approximate analyses:

## Example No. 1

|         | Per cent | 90 |
|---------|----------|----|
| Silver  | 92.5     |    |
| Cadmium | 3.5      |    |
| Tin     | 3.5      |    |
| Nickel  | 0.5      | 95 |

## Example No. 2

|         | Per cent | 100 |
|---------|----------|-----|
| Silver  | 92.5     |     |
| Cadmium | 3.5      |     |
| Tin     | 3.0      | 100 |
| Silicon | 0.5      |     |
| Nickel  | 0.5      |     |

## Example No. 3

|           | Per cent | 105 |
|-----------|----------|-----|
| Silver    | 92.5     |     |
| Cadmium   | 3.0      |     |
| Tin       | 3.0      |     |
| Nickel    | 0.5      |     |
| Magnesium | 1.0      | 110 |

The new alloys can be made in finenesses substantially less than sterling fineness and I have found that alloys of the new type as low as 800 fine can be made by using varying percentages of 5 cadmium and tin, or zinc and tin, the ratio of the cadmium or zinc to tin being increased as the silver content decreases. The quantity of the hardening elements present, however, remains substantially unchanged.

10 An example of the new alloy 800 fine may have the following approximate analysis:

*Example No. 4*

|                                         | Per cent |
|-----------------------------------------|----------|
| 15 Silver                               | 80       |
| Cadmium                                 | 14.5     |
| Tin                                     | 5        |
| Nickel, antimony, magnesium, or silicon | 0.5      |

As above mentioned, zinc may be substituted 20 for all or part of the cadmium in the 800 fine alloy, but I prefer to employ cadmium.

I am aware that it has been proposed heretofore 25 to make silver alloys which contain zinc, antimony, and tin, and tin and chromium, but after a large number of experiments involving the exposure of these alloys to various forms of tarnish, I have found that the ranges of cadmium and tin and the relative proportions used are quite critical and any substantial departure from the ranges

given results in a lowered tarnish resistance. My tests indicate further that increasing the cadmium content improves the resistance of the alloy to certain forms of tarnish while increasing the tin improves the resistance to certain other forms of tarnish. An alloy which has the best resistance for tarnish from all sources is one in which the cadmium (or zinc) and tin are present in amounts within the ranges specified for an alloy of sterling fineness.

What I claim is:

1. A silver alloy which comprises silver ranging from about 80% to 92.5%, cadmium ranging from about 14.5% to about 3%, tin ranging from about 5% to about 3% and nickel ranging from about 0.25% to about 1%.

2. A silver alloy which comprises silver ranging from about 80% to about 92.5%, cadmium ranging from about 14.5% to about 3%, tin ranging from about 5% to about 3% and about 0.5% of nickel.

3. A silver alloy of sterling fineness which comprises about 92.5% of silver, from about 4% to 3% of cadmium, from about 4.5% to about 3% of tin, and from about 0.25% to about 1% of nickel.

4. A silver alloy of sterling fineness which comprises about 92.5% of silver, about 3.5% of cadmium, about 3.5% of tin, and about 0.5% of nickel.

ROBERT H. LEACH.

30

80

85

35

90

95

40

110

45

115

50

120

55

125

60

130

65

135

70

140

75

150